

## UNITED STATES PATENT OFFICE.

ERNST SCHWARZ, OF BERLIN, AND LOUIS BLANGEY, OF MANNHEIM, GERMANY,  
ASSIGNEES TO BADISCHE ANILIN & SODA FABRIK, OF LUDWIGSHAFEN-ON-  
THE-RHINE, GERMANY, A CORPORATION.

## TANNING.

1,289,280.

Specification of Letters Patent. Patented Dec. 31, 1918.

No Drawing.

Application filed April 27, 1917. Serial No. 165,001.

To all whom it may concern:

Be it known that we, ERNST SCHWARZ and LOUIS BLANGEY, citizens of the German Empire and the Swiss Republic, respectively, residing at Berlin and Mannheim, respectively, Germany, have invented new and useful Improvements in Tanning, of which the following is a specification.

We have found that we can convert hides into a leather having good properties by treating the hides with a bath containing a carbazole sulfonic acid. Under this term we comprise the monosulfonic and polysulfonic acids of carbazole itself or of carbazole derivatives or of crude carbazole or of waste products containing carbazole as a chief constituent. The said sulfonic acids can be employed either alone or in the form of mixtures of several sulfonic acids and in either case other tanning materials or other bodies can be added. The said sulfonic acids can be directly employed in the free state or their salts, especially their alkali salts, can be used with an addition of an acid.

The following is an example of how the invention can be carried out but the invention is not confined to this example.

Dissolve 70 parts of carbazole monosulfonic acid sodium salt in 1000 parts of water, acidify with 70 parts of dilute sulfuric acid of 10%, introduce the hides de-

prived of lime by means of a bisulfite solution and treat until they are thoroughly tanned. Then the leather is washed and fatted as usual.

In an analogous manner the process can be carried out by preparing the tanning bath with other carbazole sulfonic acids, for instance such as carbazole disulfonic acid sodium salt or the mixture of sulfonic acids obtained by sulfonating pure or crude carbazole, *e. g.* the anthracene waste products obtained by purifying crude anthracene, or sulfonic acids of chlor-carbazole or N-methyl carbazole and so on.

What we claim is:

1. The process of tanning which comprises treating hides in a bath containing a carbazole sulfonic acid.

2. The process of tanning which comprises treating hides in a bath containing a plurality of carbazole sulfonic acids.

3. The process of tanning which comprises treating hides in a bath containing sulfonated crude carbazole.

4. As a new article of manufacture a leather containing as a tanning constituent a carbazole sulfonic acid.

In testimony whereof we have hereunto set our hands.

ERNST SCHWARZ.  
LOUIS BLANGEY.